

Aug. 19, 1941.

G. DE W. GRAVES

2,253,176

## METHOD AND APPARATUS FOR PRODUCTION OF STRUCTURES

Filed Aug. 9, 1938

Fig. 1.



Fig. 2.



Fig. 4.



*George De Witt Graves* INVENTOR.

BY *Louis Weisbe*  
ATTORNEY

## UNITED STATES PATENT OFFICE

2,253,176

## METHOD AND APPARATUS FOR PRODUCTION OF STRUCTURES

George De Witt Graves, Wilmington, Del., assignor to E. I. du Pont de Nemours & Company, Wilmington, Del., a corporation of Delaware

Application August 9, 1938, Serial No. 223,997

13 Claims. (Cl. 18—8)

This invention relates to the production of yarns, filaments, ribbons, and the like. More particularly, it relates to the melt spinning of yarns, filaments, ribbons, and the like from organic filament-forming compositions which have a tendency to change their chemical composition while in the molten state.

The spinning of filaments from molten filament-forming compositions is a relatively new art and presents numerous difficulties. Some of these difficulties result from the decomposition of the filament-forming compositions contemplated. This decomposition is objectionable not only because of the degradation of the filament-forming composition with its accompanying effect upon the properties of the filaments produced but also because it often results in the formation of gaseous products which form bubbles in the molten filament-forming composition. The presence of these bubbles results in filaments of non-uniform denier since the gaseous component is metered along with the molten filament-forming composition prior to extrusion. Likewise this decomposition often results in a change of viscosity of the filament-forming composition which may also result in a change in denier. Similarly, in the melt spinning of certain organic filament-forming compositions of a polymeric nature, further polymerization may occur at the temperature of melt spinning so that the viscosity is raised and other properties affected. Likewise, slight differences in the extruded filaments are likely to produce large dyeing differences in the finished product. Frequently, two or more of these effects may occur simultaneously. It is, therefore, impossible to compensate for these changes by careful control of temperature, rate of metering, pressure, rate of draw-off of the extruded filaments, etc., and obtain filaments of very uniform quality and denier.

It is, therefore, an object of this invention to provide an improved method and apparatus for the melt spinning of filaments from organic filament-forming compositions.

It is another object of this invention to provide an improved method and apparatus for the continuous melting and continuous withdrawing of organic film-forming or filament-forming compositions which have a tendency to change their chemical form while in the molten state.

It is a further object of this invention to provide an improved method and apparatus for the melt spinning of filaments from organic filament-forming compositions in which the solid composition is melted at a rapid rate.

It is a further object of this invention to provide an improved method and apparatus for the production of organic filaments from a melt with a minimum exposure of the melt to elevated temperatures.

It is another object of this invention to provide an improved method and apparatus for the continuous melt spinning of filaments, ribbons and the like from organic filament-forming compositions which have a tendency to change their chemical form while in the molten state.

Other objects of the invention will appear hereinafter.

The objects of this invention are accomplished, in general, by feeding the solid organic filament-forming composition on to a heated surface upon which melting occurs at a rate substantially equal to the rate of withdrawal of the molten composition, and allowing the molten filament-forming composition to flow to a pool of restricted volume from which the molten filament-forming composition may be withdrawn, for example, by forcing the same through an opening of a desired size and shape, solidifying the formed composition, and collecting the solidified articles in any desired manner.

In order to more clearly define the present invention, reference is made to the following detailed description taken in connection with the accompanying illustration, in which:

Figure 1 is a diagrammatic, side elevational view of an apparatus for melt spinning according to the invention.

Figure 2 is a similar view of another modification of the invention.

Figure 3 and Figure 4 are diagrammatic, side elevational views showing modified forms of the grid melting unit used in the present invention.

In Figure 1, reference numeral 11 represents a cylindrical chamber which may be insulated or which may be provided with means for heating the same. The chamber 11 is provided with a flat spiral metal coil or grid 12. The grid 12 is constructed of tubing and is preferably constructed from a non-corrosive metal such as stainless steel, Monel, illium or similar metal alloy. The spiral coil grid 12 may be heated by means of electrical resistance units positioned at the interior thereof or by means of a heating medium circulated therethrough. Solid pieces, e. g., flakes 15 of the organic filament-forming composition shown at 13 are allowed to fall, preferably at a uniform rate, from the flake hopper 14 located above the chamber. If desired, an atmosphere of an inert gas may be main-

tained in the chamber 11. These flakes come to rest on the surface of the grid 12, which is heated to a temperature above the melting point of the organic filament-forming composition. The flakes melt on the surface of the grid 12 and the molten filament-forming composition drains between the turns of the grid and is shown dropping at 16 to the pool 17 from whence it may be withdrawn in any desired manner such as by means of a pumping element, e. g., a gear metering pump, for example, a pump similar to the type commonly used in the spinning of filaments from viscose, which meters it to the spinneret from which it is forced in the form of filaments, ribbons or the like.

For the most satisfactory operation of the invention, these flakes shown at 15 should be of essentially uniform size and of somewhat larger size than the spaces between turns of the melting grid 12. This eliminates any possibility of unmelted material falling through the grid. It is to be noted, however, that once melting has begun and the viscous, molten filament-forming composition is draining through the grid, flakes do not tend to fall through unmelted even though they be somewhat smaller than the grid separation since they are caught in the viscous mass. While the separation of the turns of the grid can be varied over considerable limits depending on the size of the flakes or chips of the filament-forming composition, the minimum separation of the turns of the grid is critical and is dependent on the viscosity of the molten filament-forming composition. If the turns of the grid are too closely spaced the molten material does not drain properly. It is, therefore, necessary to provide grid turns with sufficient separations to permit proper draining of the molten filament-forming composition and to provide flakes of the solid filament-forming composition of proper size relative to the grid separation.

Not only is it important that the flakes of filament-forming composition have a certain minimum size but it is also important that they be of a uniform size and only slightly larger than the spaces between the turns of the grid. There are several reasons for this: To achieve uniform melting and minimum exposure to the elevated temperature it is desired that a maximum surface area of the flake be in contact with the melting grid, which is attained by minimum flake size; to obtain melting at a uniform rate, which is vital to the invention, the particles should be of uniform size in order that they will melt at substantially the same rate; and likewise the feeding of the flakes to the melting grid is facilitated by the use of small uniformly sized flakes. Flakes suitable for use in this invention can be conveniently prepared by a process disclosed in the applicant's copending application Serial No. 223,998 filed of even date herewith.

It is usually preferable to provide a melting unit for each spinneret since it is desired to maintain a minimum quantity of the filament-forming composition in the molten condition. It is to be understood, however, that the invention is not so limited, for by placing a plurality of spinnerets in close proximity to the melting grid, supplied by a rapid parallel or a circulating series flow through restricted passages or by other special means, one melting unit could supply a plurality of spinnerets.

While it might be expected that as each individual flake melts, and its size decreases, a solid residue would drop into the pool below unmelt-

ed, this is not the case. The viscosity and other physical properties of molten organic filament-forming compositions are such that the solid particle adheres to the grid surface until it is completely melted.

Although the rate at which the flakes are fed to the grid may be accurately adjusted to the rate of extrusion of the molten filament-forming composition, it is desirable to know the quantity of liquid material present in the pool at all times, since an object of the invention is to obtain minimum exposure of the molten material to elevated temperatures. This may be done in a number of ways as by the use of gauges, windows, and the like. A particularly convenient method of determining the quantity of liquid in the molten pool is by means of a conductivity measurement, since organic filament-forming compositions exhibit sufficient electrical conductivity for such a measurement. This may be done by inserting a vertical electrode 18 through the bottom of the melt chamber 11 by means of suitable insulation 20. This electrode is connected through a suitably calibrated milliammeter 22 to a battery 24 or other power source and thence connected to the walls of the melt chamber which comprise the other electrode. The circuit is completed through the molten filament-forming composition. A rise in level is accompanied by an accompanying increase in the flow of current.

In accordance with the present invention, it is preferred to restrict the amount of molten filament-forming composition in the pool to the minimum quantity required to continuously supply the spinneret or other extruding means. The maximum volume permissible depends to a large extent on the nature of the filament-forming composition and the rate of extrusion. In general, it is preferred that the volume does not exceed that which will be withdrawn from the pool in one hour, and more preferably in 15 minutes.

Another modification of the invention is shown in Figure 2. In this figure, reference numeral 26 represents a cylindrical chamber preferably heated internally by passing a hot vapor, e. g., steam at high pressures, or Dowtherm, through the passages represented at 28. A melting grid 30, preferably composed of metal, is heated internally, for example, by the passage therethrough of a hot vapor. The melting grid 30 is provided with a metal plate 32 covering the open space left by the last turn of the coil. The unheated cylindrical chamber 34 is filled with the flakes of filament-forming composition. The chamber 34 is preferably provided with a closure 36. In many instances, it is desired to preheat the flakes of filament-forming composition in this chamber. This increases the rate of melting when the flakes reach the grid and removes any excess moisture which may have condensed on the flake. This preheating may be accomplished by heating the chamber or in any other desired manner, but in no case should the temperature closely approach the melting point of the filament-forming composition. A hopper 38 is positioned below the grid 30. The molten filament-forming composition flows into the hopper 38 after melting on and draining through the grid 30. This molten filament-forming composition then flows from the hopper 38 through the passage 40 to the gear metering pump 42 from which it is forced to the spinneret pack 44 and spinneret 46 through conduit 48. The molten material is ex-

truded through the spinneret 48 in the form of filaments, ribbons, and the like. If it is desired to maintain an atmosphere of an inert gas in the chamber, this can be done by introducing the gas at 50 and removing it by suitable means at 52 and 54.

This modification of the invention differs from that described in Figure 1 since the melt level is automatically maintained. As a solid body of the flakes is fed to the melting grid, melting occurs and the hopper 38 becomes completely filled. Further melting results in the formation of a thin layer of the molten filament-forming composition above the melting grid. Since the heat conductivity of the molten material is very low, insufficient heat is transferred through this thin layer of molten material to melt the solid above. Consequently, no further melting occurs until sufficient molten material has been displaced by spinning to permit the level to fall 20 below the level of the grid and to permit the solid filament-forming material to come into contact with the grid. This construction of the apparatus allows the maintenance of a constant minimum quantity of the molten material. 25 When spinning at a constant rate, the molten material is discharged at a constant rate so that it is exposed to an elevated temperature for a constant minimum length of time. In this modification the minimum size of the flakes is not so 30 critical since the solid pieces tend to float and so do not get into the pool below the melting grid.

The process, with particular reference to the apparatus shown in Figure 2, will now be described more specifically with reference to the melt spinning of polyhexamethylene adipamide, a fiber-forming linear polyamide obtainable by the condensation polymerization of hexamethylene diamine and adipic acid and which has a 35 melting point of about 265° C.

Flakes of polyhexamethylene adipamide approximately  $\frac{1}{4}'' \times \frac{1}{4}'' \times \frac{1}{8}''$  were placed in the chamber 34 completely filling it and the space in the chamber 26 above the melting grid 30. The flakes rested on the melting grid, which was constructed from  $\frac{1}{8}''$  stainless steel tubing, the tubes being uniformly separated slightly less than  $\frac{1}{8}''$ . The diameter of the grid was 6''. The capacity for the flakes was approximately 20 liters. The top 38 of the chamber 34 was tightly closed and nitrogen forced in at 50 and released through suitable cocks positioned in outlets 52 and 54. This diversion of the flow of the inert gas permitted the maintenance of an inert atmosphere throughout the chamber and its passage in the proximity of the grid sweeps out any gases liberated upon melting. A pressure of 10 lbs. of  $N_2$  per square inch was maintained inside the chamber to prevent any diffusion of air into the apparatus. The flow of gas thus permitted replenishing the supply of the flakes without interrupting spinning.

The passages 28 in chamber 26 and the melting grid 30 were maintained at 285° C. The flakes in contact with the grid melted and the filament-forming composition drained into the hopper 38, through the passage 40 to the gear pump 42 which forced it to the spinneret pack 44 and spinneret 48 from which it was spun at 70 a rate of about 15 grams per minute in the form of filaments. The total volume of the pool in hopper 38, the passages 40 and 48, the pump 42, and spinneret pack 44 was approximately 200 c. c. so that sufficient molten filament-forming

composition for approximately 10 minutes' spinning was continuously maintained.

As soon as the melt pool in hopper 38 was filled, a thin layer of molten material formed on the surface of the grid 30 and due to the low heat conductivity of the molten material no further melting occurred until the level dropped to that of the grid. As a result, the flakes melted only as rapidly as the molten filament-forming composition was spun and a constant quantity of melt was automatically maintained.

In all of the modifications of the present invention, the molten filament-forming composition continuously drains from the melting surface. This downward flow of melt washes from the melting surface any stagnant film which tends to collect, thereby contributing to the uniformity of the melt and decreasing the possibility of decomposition.

While grid melting units spirally shaped and heated by electrical resistance or heated internally by circulation of a hot fluid have been described, the invention is not so limited. The grid melting unit may take the form of a hollow cone 60 formed from rods or tubing as shown in Figure 3. In this modification, it may be desirable to provide the top of the cone 60 with a cap 62. Similarly, the grid melting unit may comprise a pair of perforated metal discs 64 wedged against the side walls of the melt chamber 66, as shown in Figure 4. A plurality of tubes 68 may be arranged between the discs 64. Such discs 64 and tubes 68 can be heated by conduction of heat from the outside of the melting chamber, internally by the circulation of a hot vapor or gas or by the passage of electrical current due to their resistance. Similarly, the grids may be heated by the induced current produced in an electrostatic field.

Similarly the grid may take the form of parallel elements or elements arranged in any desired configuration to form spaces of uniform size through which the molten composition will drain, but which will prevent the passage of solid particles. Where spiral grids are used they may be formed from more than one circuit of pipe. Likewise, in some instances, it may be desirable to use more than one grid, or a second heating element may be immersed in the liquid pool to maintain it at any desired temperature.

The melting grids, in accordance with the present invention, may be maintained at any suitable temperature; preferably however, the melting grids are maintained at a temperature not to exceed 40° C. above the melting point of the filament-forming composition being spun.

While specific reference has been made to the use of a gear pump for forcing the molten filament-forming composition to the spinneret, the invention is not so limited. Use may be made of screw pumps, piston pumps, or pumps of any other type or gas pressure may be used for this purpose. If desired, use may be made of a combination of two pumps of the same or different types in series or combinations of gas pressure and pumps.

As indicated above, in many cases, it may be preferable to maintain an inert atmosphere in the melt chamber, to prevent or reduce oxidation of the molten filament-forming composition. Nitrogen, carbon dioxide, hydrogen or any other oxygen-free gas which is inert to the filament-forming composition, may be used for this purpose. The gas may be introduced at any convenient point in the melt chamber to maintain

such an atmosphere. If desired, the face of the spinneret may be similarly blanketed to prevent oxidation of the freshly extruded filaments with accompanying interruption of the spinning.

Many other variations can be made in the specific details above set forth, for example, it may be desirable under certain circumstances to melt the filament-forming material at a temperature well above the melting point and cool the molten composition before it is extruded, thus increasing the speed of melting with a minimum of decomposition.

In the foregoing description this invention has been illustrated with special reference to the spinning of polyhexamethylene adipamide but it is not so limited.

This invention is peculiarly adaptable to the spinning from melt of filaments and the like from these fiber forming synthetic linear polymers and particularly to the synthetic linear polyamides which belong to this class since these synthetic linear polymers are crystalline in the solid state as evidenced by X-ray investigation and they have a definite melting point. These synthetic linear polymers melt sharply, forming liquids which drain readily from the melting grid thus facilitating control of the melting and reducing any tendency to decompose at elevated temperatures. Other synthetic linear polymers include the polyesters, polyethers, polyacetals, mixed polyester-polyamides, etc. which, for example, may be prepared by a process of condensation polymerization as described in U. S. Patent No. 2,071,250.

My invention is also applicable to advantage in the spinning from melt of filament and the like, of the polymers prepared by the high pressure polymerization of ethylene which are more fully described in the copending application of Fawcett, Gibson and Perrin, Serial Number 123,722 filed February 2, 1937 since they are also crystalline in the solid state.

This invention is also applicable to the spinning of other organic filament forming compositions which are capable of being spun from melt particularly to the extruding of such materials which have a tendency to change their chemical composition while in their molten state. As examples of such filament forming compositions may be mentioned vinyl polymers, polystyrene and polyacrylic acid derivatives. Cellulose derivatives, e. g., cellulose acetate suitably plasticized can also be spun according to the invention.

The present invention, furthermore, is not to be limited to the spinning of ribbons and filaments; the molten material may, for example, be withdrawn for the continuous coating of articles such as wire with synthetic linear polymers whereby to electrically insulate the same.

The filament-forming material used in the process of this invention may contain modifying agents, e. g., luster modifying agents, plasticizers, pigments, dyes, antioxidants, resins, etc.

By practice of this invention, the solid filament-forming composition is melted rapidly and continuously whereupon the molten filament-forming composition drains directly to a pool of restricted volume from which it is extruded in the form of filaments, ribbons, and the like. Since the filament-forming composition is exposed to an elevated temperature for a minimum, constant period, any tendency toward decomposition, the formation of gaseous products and any tendency to polymerize further is reduced

to a minimum or is maintained at a constant rate. It is possible, therefore, to obtain in a continuous manner molten organic filament-forming compositions having uniform properties and to extrude these molten filament-forming compositions in a uniform and continuous manner in the form of yarns, filaments, ribbons, and the like. By collecting the freshly spun filaments in an orderly manner, filaments will be obtained of extremely uniform denier and of uniform physical and chemical characteristics.

Since it is obvious that many changes and modifications can be made in the above detailed description without departing from the nature and spirit of the invention, it is to be understood that the invention is not to be limited except as set forth in the appended claims.

I claim:

1. In an apparatus for the melt spinning of structures from an organic filament-forming composition, a grid having a plurality of openings therein, means for heating said grid to a temperature above the melting point of said composition, means for feeding solid particles of said composition on to said grid, means for collecting the liquid molten composition in the form of a pool, and pumping means for forcing said composition to a spinning unit.

2. In an apparatus for the melt spinning of structures from an organic filament-forming composition, a grid having a plurality of openings therein, means for heating said grid to a temperature above the melting point of said composition, means for feeding solid particles of said composition on to said grid, means for collecting the liquid molten composition in the form of a pool, and pumping means for forcing said composition to a spinning unit.

3. In an apparatus for the melt spinning of structures from an organic filament-forming composition, a grid having a plurality of openings therein, means for heating said grid to a temperature above the melting point of said composition, means for feeding solid particles of said composition on to said grid, means for collecting the liquid molten composition in the form of a pool, said grid positioned within said collecting means whereby the level of the pool may rise to cover said grid.

4. In an apparatus for the melt spinning of structures from an organic filament-forming composition, an enclosure, a grid melting unit in said enclosure, means for conducting solid organic filament-forming composition onto said unit, means through which the liquid molten composition is extruded, collecting means, intermediate said unit and extrusion means, for collecting a sufficient quantity of liquid molten composition to provide a substantially constant volume of flow of said liquid composition through said extrusion means.

5. In an apparatus for the melt spinning of structures from an organic filament-forming composition, an enclosure, a grid melting unit in said enclosure, means for conducting solid organic filament-forming composition onto said unit, means through which the liquid molten composition is extruded, collecting means, intermediate said unit and extrusion means, for collecting a sufficient quantity of liquid molten composition to provide a substantially constant volume of flow of said liquid composition through said extrusion means, said unit positioned within said collecting means whereby the level of the pool may rise to cover said unit.

6. In an apparatus as set forth in claim 4 in

which the grid is a spiral structure, the elements forming the spiral structure being spaced from each other to provide openings therebetween.

7. In an apparatus as set forth in claim 4 in which the grid is a spiral tubular structure, the elements forming the spiral structure being spaced from each other to provide openings therebetween.

8. In an apparatus for the melt spinning of structures from an organic filament-forming composition, an enclosure, a grid melting unit in said enclosure, means for conducting solid organic filament-forming composition onto said unit, means through which the liquid molten composition is extruded, collecting means, intermediate said unit and extrusion means, for collecting a sufficient quantity of liquid molten composition to provide a substantially constant volume of flow of said liquid composition through said extrusion means, conduit means connected to said solid conducting means, additional conduit means connected to said enclosure, said several conduit means adapted to pass an inert gas about said solid as the latter is conducted to the said unit.

9. In an apparatus for the melt spinning of structures from an organic filament-forming composition, an enclosure, a grid melting unit in said enclosure, means for conducting solid organic filament-forming composition onto said unit, means through which the liquid molten composition is extruded, collecting means, intermediate said unit and extrusion means, for collecting a sufficient quantity of liquid molten composition to provide a substantially constant volume of flow of said liquid composition through said extrusion means, and inert gas conveying means connected to said solid conducting means and said enclosure for sweeping objectionable gaseous elements from said enclosure.

10. In an apparatus as defined in claim 1, means for maintaining an inert gas in contact with the melting and melted composition.

11. In a process for the melt spinning of a yarn from a molten synthetic linear polyamide spinning composition, the steps comprising continuously melting small solid particles of said composition in an atmosphere consisting of a gas inert to said composition, and continuously extruding the molten composition, the melting and extruding of the composition being carried out at a temperature not to exceed 40° C. above the melting point of the composition, and the melting of said composition being carried out at a rate substantially equal to the rate of extrusion of said composition.

12. In a process for the melt spinning of structures from a molten organic filament-forming composition, the steps comprising passing small, solid particles of said composition on to a heated surface to melt the same, passing an oxygen-free gas through said particles, extruding the resulting molten composition, the melting of said composition being carried out at a rate substantially equal to the rate of extrusion of molten composition.

13. In a process for the melt spinning of structures from a molten organic filament-forming composition, the steps comprising passing small, solid particles of said composition on to a heated surface to melt the same, passing an oxygen-free gas in a plurality of paths through said particles, extruding the resulting molten composition, the melting of said composition being carried out at a rate substantially equal to the rate of extrusion of molten composition.

GEORGE DE WITT GRAVES.